

# United States Patent [19]

Swanson

[11] 3,804,677

[45] Apr. 16, 1974

[54] **WORKING OF ALLOYS**

[75] Inventor: **Colin John Swanson, Bristol, England**

[73] Assignee: **ISC Alloy Limited of Austral House, London, England**

[22] Filed: **Nov. 6, 1972**

[21] Appl. No.: **303,718**

[30] **Foreign Application Priority Data**

Nov. 4, 1971 Great Britain ..... 51322/71

[52] **U.S. Cl.** ..... 148/11.5 R

[51] **Int. Cl.** ..... C22f 1/16

[58] **Field of Search** ..... 148/11.5 R

[56] **References Cited**

UNITED STATES PATENTS

3,420,717 1/1969 Fields, Jr. et al. 148/11.5 R

3,567,524 3/1971 Cook et al. ..... 148/11.5 R

*Primary Examiner*—W. W. Stallard

*Attorney, Agent, or Firm*—Holman & Stern

[57] **ABSTRACT**

A process for working superplastic sheet material comprising shaping the superplastic alloy by pressure or vacuum forming, annealing the sheet material before or after the pressure of vacuum forming, and bending at least a part of the shaped sheet at room temperature. In a preferred procedure rolled superplastic zinc/aluminium alloy sheet material is annealed at about 200° C for at least one hour, vacuum or pressure forming carried out at 200° C to 250° C after the annealing, and the shaped sheet allowed to cool to room temperature before bending.

**10 Claims, No Drawings**

## WORKING OF ALLOYS

This invention relates to the working of alloys which can be conditioned to exhibit the phenomenon known as superplasticity, and in particular to the working of superplastic zinc/aluminium alloys.

The term superplasticity as used in this specification relates to the condition in which alloys exhibit a substantial strain rate sensitivity. Strain rate sensitivity, denoted  $m$ , is the exponential variable in the expression  $\alpha = K\xi^m$ , wherein  $\alpha$  represents stress in load per unit area,  $\xi$  represents strain rate in terms of length change per unit time, and  $K$  represents a constant which is termed the strain rate co-efficient.

While the existence of a substantial strain rate sensitivity  $m$  determines the ultimate elongation to which an alloy may be subjected without fracture, the strain rate coefficient  $K$  is significant in determining the strength of the material and hence the amount of work which must be put in to achieve a given forming operation.

It is already known to condition a blank of alloy to exhibit superplasticity by means of a heat treatment/quenching/working technique and to cause the blank thus conditioned to conform to the shape of a moulding surface by means of fluid pressure or vacuum. However, after this moulding operation the alloy may still require further working to produce a further shape feature, for example a flange may be required on the finished article and this may involve a bending operation on at least a part of the moulded shape.

It may be demonstrated that the desirable properties of superplastic alloys may be achieved only at the expense of a reduction in the capability of the material to withstand bending stresses without cracking.

Because superplastic alloys are characterized by their high degree of strain rate sensitivity it is clear that difficulties encountered during cold bending may be overcome by lowering the rate of such bending. While this expedient may be acceptable in limited instances it is unlikely to be acceptable in a commercial forming process.

The invention in one aspect consists in a process for working alloy sheet material which has been conditioned to exhibit superplasticity, comprising: shaping the superplastic alloy by pressure or vacuum forming; annealing the sheet material before or after the said pressure or vacuum forming; and bending at least a part of the shaped sheet at or near room or ambient temperature. Room or ambient temperature is to be understood to be about 20° C.

Usually the annealing is carried out before the vacuum or pressure forming operation.

Preferably the annealing temperature is within the range 150° to 250° C, more preferably about 200° C.

The annealing time is suitably 1 to 2 hours.

In a preferred procedure rolled superplastic zinc/aluminium alloy sheet material is annealed at about 200° C for at least 1 hour, vacuum or pressure forming carried out at 200° C to 250° C, and the shaped sheet allowed to cool to room temperature before bending.

The invention in another aspect consists in a process for working an alloy sheet material comprising rendering the alloy superplastic (as hereinbefore described), shaping the superplastic alloy by pressure or vacuum forming, annealing the sheet material before or after the said pressure or vacuum forming, and bending at

least a part of the shaped sheet at or near room or ambient temperature.

The invention will be further described with reference to the following examples.

Tables 1, 2 and 3 below show the results of bending strips of a zinc/aluminium alloy (containing 87% by weight of zinc, 22% aluminium, and 0.15% of copper as a ternary element) of dimensions 1 1/4 inches × 3 1/4 inches around different bend radii (in inches) for three different gauges of alloy sheet, i.e. 0.025 inches, 0.050 inches, and 0.075 inches gauge. The specimens were annealed for 1 hour at 200° C and 250° C and then bent cold around the specified radii. The results of the cold bend tests are shown in the Tables.

The rating of the effect of bending is related to the following scale:

| Rating | Degree of Cracking |
|--------|--------------------|
| 1      | Complete fracture  |
| 3      | Heavy cracking     |
| 5      | Moderate cracking  |
| 7      | Light cracking     |
| 9      | No cracks.         |

It will be appreciated that even-number bend ratings indicate intermediate degrees of cracking, i.e. degrees of cracking between those indicated by the odd-number ratings.

Table 1

| 0.025 inch Gauge Sheet |                       |     |                         |
|------------------------|-----------------------|-----|-------------------------|
| Bend Radius (Inches)   | As Rolled             |     | Anneal Temperature (°C) |
|                        | (at room temperature) | 200 | 250                     |
| 0.250                  | 9                     | 9   | 9                       |
|                        | 9                     | 9   | 9                       |
|                        | 9                     | 9   | 9                       |
|                        | 9                     | 9   | 9                       |
|                        | 6                     | 9   | 9                       |
|                        | 6                     | 8   | 9                       |

Table 2

| 0.050 inch Gauge Sheet |                       |     |                         |
|------------------------|-----------------------|-----|-------------------------|
| Bend Radius (Inches)   | As Rolled             |     | Anneal Temperature (°C) |
|                        | (at room temperature) | 200 | 250                     |
| 0.250                  | 9                     | 9   | 9                       |
|                        | 5                     | 9   | 9                       |
|                        | 1                     | 5   | 5                       |
|                        | 1                     | 5   | 5                       |
|                        | 1                     | 5   | 5                       |
|                        | 1                     | 5   | 6                       |

Table 3

| 0.075 inch Gauge Sheet |                                 |                         |     |
|------------------------|---------------------------------|-------------------------|-----|
| Bend Radius (Inches)   | As Rolled (at room temperature) | Anneal Temperature (°C) |     |
|                        |                                 | 200                     | 250 |
| 0.250                  | 9                               | 9                       | 9   |
| 0.125                  | 5                               | 5                       | 5   |
| 0.080                  | 3                               | 4                       | 4   |
| 0.040                  | 4                               | 5                       | 5   |
| 0.020                  | 4                               | 4                       | 4   |
| 0                      | 3                               | 4                       | 4   |

Although raising the annealing temperature to 250° C results in some further improvement in bending performance, practical difficulties may arise due to distortion of the formed component. That the temperature of annealing should be of the order of 200° C is illustrated in Table 4 in which sheet material 0.05 inches thick of a zinc/aluminium alloy (containing 70% by weight of zinc, 30% aluminium, and 0.01% of magnesium as a ternary element) was annealed for 24 hours at various temperatures prior to cold bending.

Table 4

| Bend Radius (inches) | As Rolled (at room temperature) | Effect of temperature |     |     |     |
|----------------------|---------------------------------|-----------------------|-----|-----|-----|
|                      |                                 | 100                   | 150 | 200 | 250 |
| .250                 | 1                               | 1                     | 8   | 9   | 9   |
| .125                 | 1                               | 1                     | 7   | 9   | 9   |
| .080                 | 1                               | 1                     | 1   | 6   | 8   |
| .040                 | 1                               | 1                     | 1   | 4   | 7   |
| .020                 | 1                               | 1                     | 1   | 4   | 7   |
| 0                    | 1                               | 1                     | 1   | 4   | 7   |

It will be recognised that to some extent the improvement in cold bending which is achieved by prior annealing arises from grain growth in the superplastic alloy. Increasing grain growth detracts from the superplastic properties. However, annealing for one hour at 200° C is likely to have a negligible effect on such superplastic properties.

I claim:

1. A process for working alloy sheet material which has been conditioned to exhibit superplasticity, comprising: taking the said alloy sheet material; causing the said sheet material to conform to a moulding surface to shape the alloy sheet material; annealing the sheet material after the said shaping; and bending at least a part of the shaped sheet at room temperature.

2. A process as claimed in claim 1 wherein the annealing temperature is within the range 150° to 250° C.

3. A process as claimed in claim 1 wherein the annealing time is from 1 to 2 hours.

4. A process as claimed in claim 1 wherein the material being worked is superplastic zinc/aluminium alloy sheet material.

5. A process for working alloy sheet material which has been conditioned to exhibit superplasticity, comprising: taking the said alloy sheet material; annealing the said sheet material; causing the sheet material to conform to a moulding surface to shape the alloy sheet material after the said annealing; and bending at least a part of the shaped sheet at room temperature.

6. A process as claimed in claim 5 wherein the annealing temperature is within the range 150° to 250° C.

7. A process as claimed in claim 5 wherein the annealing time is from 1 to 2 hours.

8. A process as claimed in claim 5 wherein the material being worked is superplastic zinc/aluminium alloy sheet material.

9. A process for working alloy sheet material which has been conditioned to exhibit superplasticity, comprising: taking the said alloy sheet material; annealing the said sheet material at about 200° C for at least 1 hour; causing the said sheet material to conform to a moulding surface to shape the alloy sheet material after the said annealing, the said shaping being carried out at a temperature of from 200° to 250° C; allowing the shaped sheet to cool to room temperature; and bending at least a part of the shaped sheet at room temperature.

10. A process as claimed in claim 9 wherein the material being worked is superplastic zinc/aluminium sheet material.

\* \* \* \* \*